

## UNITED STATES PATENT OFFICE

2,135,336

## COPPER BASE ALLOY

Franz E. Hensel and Earl I. Larsen, Indianapolis,  
Ind., assignors to P. R. Mallory & Co., Inc.,  
Indianapolis, Ind., a corporation of Delaware

No Drawing. Application April 20, 1937,  
Serial No. 137,986

5 Claims. (Cl. 75—160)

This invention relates to copper alloys.

An object of the invention is to produce high strength copper alloys of good electrical and thermal conductivity.

5 Another object is to improve the electrical and heat conductivities of such alloys.

Other objects of the invention will be apparent from the following description taken in connection with the appended claims.

10 Alloys of copper which are improved by adding an element having the characteristics of cobalt have been known for some time although they have never found great commercial use. One of the reasons for this is that such alloys could not 15 be produced with consistently high physical properties in the "as cast" condition. The alloys seem to be susceptible to intercrystalline cracking and after heat treatment sand castings show very low tensile strength even though the hardness 20 might be sufficiently high. To prove satisfactory in actual service conditions it is necessary that alloys be prepared which are uniform and consistent as far as tensile, impact, fatigue and electrical properties are concerned.

25 It was furthermore found that the straight copper cobalt alloys when melted are extremely susceptible to temperature conditions and furnace atmosphere conditions as encountered in ordinary melting procedures. If the alloy is not

30 very carefully prepared and melted under strictly controlled conditions the resultant casting or forging is liable to severe cracking and therewith low tensile, impact and fatigue strength. The present invention contemplates the provision of 35 a new and improved alloy of the copper-cobalt type which is free of the shortcomings mentioned above.

The present invention comprises a combination of elements, methods of manufacture and the product thereof, brought out and exemplified in the disclosure hereinafter set forth, the scope of the invention being indicated in the appended claims.

40 The alloy of the present invention consists of copper and cobalt, beryllium and silicon. In the formation of the alloy it is permissible to provide a composition of the materials above specified in the following proportions by weight.

Per cent

50 Cobalt .1 to 10  
Silicon .05 to 5  
Beryllium .05 to 2.5  
Copper Balance.

55 We have found that in the range given above

there exist at least three types of alloys each of which may be preferable for certain uses: One type contains a higher percentage of beryllium than cobalt and silicon, the second type contains a higher percentage of cobalt than beryllium and silicon and the third type contains approximately equal percentages of cobalt and beryllium plus silicon. The preferred ranges of composition of the alloys of the three types are given below:

|           | Per cent    | 10 |
|-----------|-------------|----|
| Cobalt    | .3 to 1     |    |
| Silicon   | .1 to .5    |    |
| Beryllium | 1.25 to 2.5 |    |
| Copper    | Balance.    | 15 |

|           | Per cent  | 20 |
|-----------|-----------|----|
| Cobalt    | 1 to 3    |    |
| Silicon   | .2 to 1   |    |
| Beryllium | .1 to .75 |    |
| Copper    | Balance.  |    |

|           | Per cent   | 25 |
|-----------|------------|----|
| Cobalt    | .15 to .75 |    |
| Silicon   | .05 to .25 |    |
| Beryllium | .10 to .50 |    |
| Copper    | Balance.   |    |

30 Our tests have shown that alloy (I) will retain its hardness at much higher temperatures than straight copper-beryllium alloys. In copper-beryllium alloys the beryllium is precipitated at comparatively low temperature in the form of copper-beryllium compound.

35 The above facts are clearly illustrated by the following tables showing the change of hardness and conductivity during aging and the effect of temperature on the hardness after heat treatment of an alloy composed of 2% beryllium, 17% cobalt, .2% silicon and balance copper.

40 TABLE NO. 1  
45 Hardness vs. aging time (material quenched from 800° C.)

| Time aged | Aging tem-<br>perature<br>°C. | Brinell hard-<br>ness | 50 |
|-----------|-------------------------------|-----------------------|----|
| 1 hour    | 350                           | 422                   |    |
| 2 hours   | 350                           | 422                   |    |
| 4 hours   | 350                           | 430                   |    |
| 8 hours   | 350                           | 422                   |    |
| 16 hours  | 350                           | 401                   |    |

55

TABLE NO. 2

Conductivity vs. aging time (material quenched from 300° C.)

| Time aged | Aging temperature | Electrical conductivity |         |
|-----------|-------------------|-------------------------|---------|
|           |                   | °C.                     | Percent |
| 10 hours  | 350               | 16.3                    |         |
| 2 hours   | 350               | 23.7                    |         |
| 4 hours   | 350               | 25.6                    |         |
| 8 hours   | 350               | 26.2                    |         |
| 16 hours  | 350               | 27.0                    |         |

15

TABLE NO. 3

Hardness vs. temperature (material aged 16 hours at 350° C.)

| Time heated after aging | Temperature | Brinell hardness |  |
|-------------------------|-------------|------------------|--|
|                         |             | °C.              |  |
| 0 hours                 | 350         | 430              |  |
| 2 hours                 | 400         | 415              |  |
| 2 hours                 | 450         | 390              |  |
| 2 hours                 | 500         | 280              |  |
| 2 hours                 | 500         | 225              |  |

30 Alloys of the type (II) require a much higher temperature for precipitation and are about the highest temperature resisting alloys on a copper base. By adding such ingredients as silicon and cobalt, to a copper-beryllium alloy, the precipitation is retarded at low temperatures and the strength is still maintained after heating at a temperature of several hundred degrees above the softening point of binary copper-beryllium alloys.

35 The improvements in the secondary type of an alloy composed of 2.3% cobalt, .4% silicon, .25% beryllium and balance copper are illustrated in Tables 4, 5 and 6.

TABLE NO. 4

45 Hardness vs. aging time (material quenched from 900° C., 950° C., and 1000° C.)

| Time aged | Aging temperature | Brinell hardness for material previously quenched from— |         |           |
|-----------|-------------------|---------------------------------------------------------|---------|-----------|
|           |                   | 900° C.                                                 | 950° C. | 1,000° C. |
| 1/4 hour  | 470               | 80                                                      | 95      | 130       |
| 1 hour    | 470               | 90                                                      | 150     | 250       |
| 2 hours   | 470               | 190                                                     | 230     | 265       |
| 3 hours   | 470               | 230                                                     | 250     | 260       |

TABLE NO. 5

Conductivity vs. aging time (material quenched from 900° C., 950° C., and 1000° C.)

| Time aged | Aging temperature | Percent conductivity for material previously quenched from— |         |           |
|-----------|-------------------|-------------------------------------------------------------|---------|-----------|
|           |                   | 900° C.                                                     | 950° C. | 1,000° C. |
| 1/4 hour  | 470               | 35                                                          | 25      | 24        |
| 1/2 hour  | 470               | 45                                                          | 34      | 34        |
| 2 hours   | 470               | 48                                                          | 43      | 40        |
| 16 hours  | 470               | 55                                                          | 50      | 45        |

75

TABLE NO. 6

Physical properties of sand cast alloy (quenched from 950° C., aged 16 hours at 450° C.)

|                       |         |        |
|-----------------------|---------|--------|
| Ultimate strength     | psi     | 93,750 |
| Elongation in 2"      | percent | 10     |
| Conductivity          | do      | 51     |
| Hardness (Rockwell B) | do      | 98-100 |

As can be seen, excellent physical properties and electrical properties are obtained.

The improvements in the third type of an alloy composed of cobalt .51%, beryllium .28%, silicon .13%, copper balance, are given below.

#### A. Hardness:

Quenched from 950° C. and aged 2 hours at 15 400° C.: 235 Brinell

#### B. Conductivity (completely heat treated): 47%

By comparing our new alloys as exemplified above it may be seen, with a straight copper-cobalt alloy in a fully heat-treated condition, our new alloy will have a tensile strength which is at least 25,000 to 60,000 psi higher than the alloy without the silicon and beryllium. The hardness is increased at the same time by at least 100 Brinell numbers. The ratio of increase in tensile properties exceeds the increase in hardness, a fact which is of extreme importance in industrial applications. It is evident that in many castings the sections can be decreased and weight can be saved by using our new and improved alloy. If these parts have to conduct electricity and heat this reduction in area will not hinder the current or heat flow since our new alloys have also a higher electrical and heat conductivity than the alloys previously used.

The heat treatment of the three types of alloys is slightly different. In type (I) where a high percentage of beryllium is present somewhat lower quenching and aging temperatures are employed than with types (II) and (III) where only a small percentage of beryllium is added. In both cases the quenching temperatures will be above 700° C. and the aging temperatures below 700° C.

The alloys may contain manganese and nickel up to .5%. Likewise the alloys may contain small proportions of other ingredients which do not materially alter their properties.

The alloy of the present invention is suitable for a variety of electrical and other uses and particularly for electric contacting members such as resistance welding electrodes, trolley wires, trolley shoes, commutator bars and the like. The alloys having in the order of 99% copper are generally preferred where the strength and hardness is sufficient because of their generally higher electrical conductivity.

While the present invention as to its objects and advantages has been described herein as carried out in specific embodiments thereof, it is not desired to be limited thereby, but it is intended to cover the invention broadly within the spirit and scope of the appended claims.

What is claimed is:

- An alloy composed of: Per cent  
Cobalt .1 to 10  
Silicon .05 to 5  
Beryllium .05 to 2.5  
Copper Balance 70
- An alloy composed of: Per cent  
Cobalt .3 to 1  
Silicon .1 to .5  
Beryllium 1.25 to 2.5  
Copper Balance 75

## 3. An alloy composed of:

|             |          |           |
|-------------|----------|-----------|
| Cobalt      | Per cent | 1 to 3    |
| Silicon     | Per cent | .2 to 1   |
| 5 Beryllium | Per cent | .1 to .75 |
| Copper      | Per cent | Balance   |

4. An alloy composed of about 99% copper  
and—

|           |          |            |
|-----------|----------|------------|
| 10 Cobalt | Per cent | .15 to .75 |
| Silicon   | Per cent | .05 to .25 |
| Beryllium | Per cent | .10 to .5  |

5. An electric contacting member suitable for  
use as resistance welding electrodes and the like  
formed of an alloy composed of:

|           |          |            |   |
|-----------|----------|------------|---|
| Cobalt    | Per cent | .1 to 10   | 5 |
| Silicon   | Per cent | .05 to 5   |   |
| Beryllium | Per cent | .05 to 2.5 |   |
| Copper    | Per cent | Balance    |   |

characterized by the combination of high 10  
strength, high hardness and high electrical con-  
ductivity.

FRANZ R. HENSEL.  
EARL I. LARSEN.